# EUROPEAN PATENT SPECIFICATION

(11) **EP 1 449 956 B1**
(45) Date of publication and mention of the grant of the patent: **28.03.2007**
(21) Application number: 04250662.6
(22) Date of filing: 06.02.2004
(51) Int. Cl.: D06P 1/66, D06P 5/00, D06Q 1/02

(54) **Process for producing synthetic fiber fabric having translucent printing (dyeing) patterns and fabric thus obtained**
Verfahren zur Herstellung von synthetischen Fasergeweben mit durchscheinenden Druck (Farb) -mustern und das so erhaltene Gewebe
Procédé de production d'un tissu de fibres synthetiques ayant des motifs d'impression translucides et produit obtenu

(30) Priority: 09.02.2003 CN 03102522
(43) Date of publication of application: 25.08.2004
(73) Proprietor: Formosa Taffeta Co.,Ltd., Touliu City, Yunlin Hsien (TW)
(72) Inventor: Chen, Young-Chin, Touliu City, Yunlin Hsien, Taiwan (TW)
(74) Representative: Sexton, Jane Helen

(56) References cited:
- DE-A- 1 619 670
- DE-B- 1 140 544

## Description

The subject invention relates to a process for producing a synthetic fiber fabric having translucent printing (dyeing) patterns thereon. The present application also describes a synthetic fiber fabric having translucent printing (dyeing) patterns thereon.

In prior art, the technique of etching a printing pattern is only applied to natural cellulose fiber products, wherein the cellulose fiber is etched by an acid to form patterns thereon. There is no commercially available synthetic fiber fabric having translucent printing (dyeing) patterns thereon. Generally, the use of the conventional printing (dyeing) process in a synthetic fiber fabric is merely to print patterns thereon. The conventional printing (dyeing) process mainly comprises the steps of presetting, etching (reducing the cellulose fiber), dyeing, printing, drying, fixing, soaping, and final treatment. The etching step is directed to render the fiber surfaces uneven by using an etching agent so as to improve the properties of the fiber such as feel. However, the conventional processes cannot provide a synthetic fiber fabric having translucent printing (dyeing) patterns thereon.

Accordingly, a process for producing a synthetic fiber fabric having translucent printing (dyeing) patterns thereon is highly desired.

The present invention relates to a process for producing a synthetic fiber fabric having translucent printing (dyeing) patterns thereon. In particular, the present invention provides a process for producing a synthetic fiber fabric having a translucent printing pattern thereon, said process comprising a printing step prior to an etching step, wherein the printing step comprises printing onto a surface of the fabric a paste for dyeingand/or printing, said paste comprising a transparent printing developer which is a quaternary ammonium salt.

The present application also describes a synthetic fiber fabric having translucent printing (dyeing) patterns thereon.

By way of illustration and to provide a more complete appreciation of the present invention with many of the attendant advantages thereof, the following detailed description is given concerning a process for producing a synthetic fiber fabric having translucent printing (dyeing) patterns thereon and a synthetic fiber fabric having translucent printing (dyeing) patterns thereon.

The present invention relates to a process for producing a synthetic fiber fabric having translucent printing (dyeing) patterns thereon. The process comprises a printing step conducted prior to an etching step and the printing step comprises printing a paste for dyeing and/or printing comprising a transparent printing developer onto a surface of the fabric. Specifically, the process comprises the steps of presetting, printing, drying, fixing, etching, soaping, dyeing and final treatment. Optionally, the order of the steps can be adjusted or additional steps can be applied therebetween if the adjustment of order or the additional steps would not result in a negative influence on the desired translucent effect of the patterns. For example, a sanding step can be applied between the presetting step and printing step, the dyeing step can be replaced by a dyeing & printing step. Furthermore, the dyeing step can be conducted prior to the dyeing & printing step or the dyeing & printing step can be conducted prior to the dyeing step.

In the printing step, a transparent printing developer is mixed with a paste for dyeing and/or printing in suitable amounts and the mixture is printed onto a surface of a fabric to form printing patterns thereon. In the etching step, the transparent printing developer accelerates the etching homogeneously. Hence, the fabric surface containing the transparent printing developer has a special etching effect and a difference in transparence from those of fabric surfaces that do not contain the transparent printing developer. Hence, patterns having special translucent effects are formed on the fabric.

The synthetic fibre fabric may be made from fibres which are not natural cellulose fibres. Examples of the materials from which the synthetic fibers may be made include, but are not limited to, polyester (such as a cationic dyeable polyester), polyamide, polypropylene, acrylic fiber, and acrylonitrile.The steps of the process of the invention are described as follows.

### Presetting

A greige is scoured and delivered to a presetting machine to preset the greige to form a fabric. The speed of the presetting machine can be, for example, from 15 to 120 meter/min. The temperature of the presetting machine can be, for example, 100 to 210°C.

### Printing, drying, fixing

The fabric is treated in a printing machine, for example, a roller-printing machine or an automatic screen-printing machine. A transparent printing developer is mixed with a paste for dyeing and/or printing in suitable amounts (for example, the amount of the transparent printing developer is 1 to 50 weight percent, preferably 3 to 15 weight percent, based on the total of the transparent printing developer and paste) to form a paste mixture. The paste mixture is printed onto the surface of the fabric at a speed of 5 to 150 meter/min to form a printing pattern on the fabric. The fabric is dried at a temperature from 50°C to 210°C and fixed at a temperature from 100°C to 210°C to render the printing pattern containing the transparent printing developer and paste bonded to the fabric surface.

The transparent printing developer used in the invention is a quaternary ammonium salt ion promoter. Persons skilled in the art can select a suitable quaternary ammonium salt as a promoter for the etching agent, for example, tetraalkyl ammonium iodide (NR₄I) and tetraalkyl ammonium hydroxide (NR₄OH) where each R is independently an alkyl or aryl group of up to 15 carbon atoms, preferably 1 to 10, more preferably 1 to 6 carbon atoms, e.g. methyl, ethyl, propyl or butyl. Generally, a quaternary ammonium salt is used as a promoter in the etching step involved in conventional dyeing and finishing processes to accelerate etching. However, conventional dyeing and finishing process does not produce a printing (dyeing) fabric having translucent patterns thereon. In other words, a quaternary ammonium salt is merely used in the conventional dyeing and finishing process to promote the etching, but not to produce a printing (dyeing) fabric having translucent patterns thereon.

### Etching

The synthetic fiber fabric having the transparent printing developer-containing paste is treated by a suitable etching agent in a suitable concentration (for example, 1 to 50 Be, preferably 15 to 35 Be) under suitable conditions, for example at a speed of 5 to 120 meter/min and at a temperature of 20°C to 150°C. The synthetic fiber fabric thus treated has a translucent printing (dyeing) pattern on the surface of the fiber to obtain a special translucent effect.

Persons skilled in the art can select suitable etching agents to effect etching. The etching agents include, but are not limited to, sodium hydroxide, sodium carbonate and sodium hydrogen carbonate.

### Soaping

The synthetic fiber fabric is then subjected to a soaping step, for example at a speed of 1200 yards/piece, to remove the impurities and processing agents on the fabric. The soaping conditions include, but are not limited to, a soaping temperature of 4°C to 120°C and a speed of 20 to 120 meter/min.

### Dyeing

The synthetic fiber fabric is dyed with suitable dyes, for example, acid dyes, disperse dyes, cationic dyes, reactive dyes, indanthrene dyes (vat) and direct dyes together with suitable dyeing auxiliaries in, for example, an air flow dyeing machine, a jigger dyeing machine, a winch dyeing machine, a beam dyeing machine, a jet dyeing machine, a rapid dyeing machine or a continuous dipping & padding dyeing machine under, for example, a temperature of 40°C to 170°C.

The synthetic fiber fabric, which is dyed or not dyed, is subjected to a dyeing & printing step. The synthetic fiber fabric is treated by suitable dyes, pigments, gold powder, silver powder, and a printing paste in a roller printing machine or automatic screen printing machine to conduct dyeing & printing under conditions, for example a speed of 15±5 meter/min. Suitable dyes include, for example, acid dyes, disperse dyes, cationic dyes, reactive dyes, indanthrene dyes (vat) or direct dyes. Alternatively, the dyeing & printing can be replaced by a transfer printing.

Either the dyeing step or dyeing & printing step, or both, can be used as desired to practice the invention. In the latter case, the dyeing step and the dyeing & printing step can be subsequently used in any order.

### Final treatment

The synthetic fiber fabric can be optionally subjected to a final treatment, for example softening, water-repelling, cold-hot calender, coating, lamination, and special waterproofing. For example, the synthetic fiber fabric can be delivered to a tank containing a softening agent to conduct the softening treatment or to a tank containing a water-repellent agent to conduct the water-repelling treatment. Then, the synthetic fiber fabric is delivered to a machine at a suitable speed (for example 35 to 55 meter/min), a suitable height (60 to 100 mm, for example 80 mm), a suitable angle (0.75 to 1.05 mm, for example, 0.95 mm), a suitable temperature (110°C to 130°C, for example 120°C) to conduct the waterproofing treatment. The synthetic fiber fabric is then stored for a suitable period of time to effect crosslinking. The fabric can be optionally subjected to a final setting to obtain the final product.

The following example is provided to further explain the invention from which the artisans can further appreciate the invention. However, the example should not be considered as a limitation to the scope of the invention.

### EXAMPLE

A greige of 450±50 yards/piece is subjected to a scouring treatment wherein the temperature of the scouring liquid is about 90±5°C and the speed is 50±10 meter/min. After scouring treatment, the greige is delivered to a presetting machine to form a fabric at a speed of 80±5 meter/min and at a temperature of 200±5°C. A printing paste containing a transparent printing developer, tetraalkyl ammonium hydroxide (NR₄OH), in which the amount of the transparent printing developer is 3 to 15 weight percent, based on the total of the transparent printing developer and paste, is printed on the fabric in a roller printing machine or automatic screen printing machine at a speed of 15±5 meter/min to form a desired printing pattern on the fabric. The fabric is then dried at a temperature of 110±10°C and fixed at a temperature of 160±20°C. The fabric is further subjected to an etching treatment in a tank having an etching agent (sodium hydroxide) with a concentration of 15 to 35 Be at a speed of 30±10 meter/min and at a temperature of 100°C ±15°C to form a printing fabric having a translucent pattern thereon. The fabric is soaped at 450±50 yards/piece at a temperature of 100°C±20°C and at a speed of 50±10 meter/min. The fabric is then dyed at a temperature of 100°C ±30°C with a dye including a dyeing auxiliary. The fabric is delivered to a tank containing a water-repellant agent to conduct a water-repelling treatment. The fabric is then delivered to a waterproofing machine at a speed of 45±5 meter/min, with a height of 80 mm, a angle of 0.95mm, a temperature of 120°C to conduct a waterproofing treatment. Then, the fabric is stored for a period of 16 hours to effect crosslinking. The fabric is subjected to a final setting conducted under a temperature of 130°C, a width of 66 inches, and a speed of 60±10 meter/min to obtain a final product.

The present embodiments are to be considered in all respects as an illustration and are not restrictive.

## Claims

1. A process for producing a synthetic fiber fabric having a translucent printing pattern thereon, said process comprising a printing step prior to an etching step, wherein the printing step comprises printing onto a surface of the fabric a paste for dyeing and/or printing, said paste comprising a transparent printing developer which is a quaternary ammonium salt.

2. A process according to claim 1 in which the quaternary ammonium salt is a tetraalkyl ammonium iodide or tetraalkyl ammonium hydroxide.

3. A process according to claim 1 or 2 in which the amount of transparent printing developer in the paste for dyeing and/or printing is 1 to 50 weight percent based on the total weight of the paste.

4. A process according to claim 3 in which the amount of transparent printing developer is 3 to 15 weight percent based on the total weight of the paste.

5. A process according to any one of the preceding claims, wherein an etching agent used in the etching step is sodium hydroxide, sodium hydrogen carbonate or sodium carbonate.

6. A process according to any one of the preceding claims wherein the process after the etching step comprises a step of dyeing and/or dyeing and printing.

7. A process according to any one of the preceding claims comprising the steps of presetting, printing, drying, fixing, etching, soaping, dyeing and final treatment.

## Patentansprüche

1. Verfahren zur Herstellung eines synthetischen Fasertuchs mit einem durchscheinenden Druckmuster darauf, wobei das Verfahren einen Druckschritt vor einem Ätzschritt umfasst, der Druckschritt das Aufdrucken einer Paste zum Färben und/oder Drucken auf eine Oberfläche des Tuchs umfasst, wobei die Paste einen transparenten Druckentwickler umfasst, der ein quaternäres Ammoniumsalz ist.

2. Verfahren nach Anspruch 1, wobei das quaternäre Ammoniumsalz ein Tetraalkylammoniumiodid oder ein Tetraalkylammoniumhydroxid ist.

3. Verfahren nach Anspruch 1 oder 2, wobei die Menge an transparentem Druckentwickler in der Paste zum Färben und/oder Drucken 1 bis 50 Gewichtsprozent, bezogen auf das Gesamtgewicht der Paste, beträgt.

4. Verfahren nach Anspruch 3, wobei die Menge an transparentem Druckentwickler 3 bis 15 Gewichtsprozent, bezogen auf das Gesamtgewicht der Paste, beträgt.

5. Verfahren nach einem der vorhergehenden Ansprüche, wobei ein im Ätzschritt verwendetes Ätzmittel Natriumhydroxid, Natriumhydrogencarbonat oder Natriumcarbonat ist.

6. Verfahren nach einem der vorhergehenden Ansprüche, wobei das Verfahren nach dem Ätzschritt einen Schritt des Färbens und/oder Färbens und Druckens umfasst.

7. Verfahren nach einem der vorhergehenden Ansprüche, umfassend die Schritte Vorfixieren, Drucken, Trocknen, Fixieren, Ätzen, Seifen, Färben und Endbehandeln.

## Revendications

1. Procédé de production d'un tissu de fibres synthétiques ayant un motif d'impression translucide dessus, ledit procédé comprenant une étape d'impression antérieure à une étape de gravure, dans lequel l'étape d'impression comprend l'impression sur une surface du tissu d'une pâte pour teindre et/ou imprimer, ladite pâte comprenant un révélateur d'impression transparent qui est un sel d'ammonium quaternaire.

2. Procédé selon la revendication 1, dans lequel le sel d'ammonium quaternaire est un iodure de tétraalkyle ammonium ou un hydroxyde de tétraalkyle ammonium.

3. Procédé selon la revendication 1 ou 2, dans lequel la quantité de révélateur d'impression transparent dans la pâte pour teindre et/ou imprimer est de 1 à 50 pourcent en poids sur la base du poids total de la pâte.

4. Procédé selon la revendication 3, dans lequel la quantité de révélateur d'impression transparent est de 3 à 15 pourcent en poids sur la base du poids total de la pâte.

5. Procédé selon l'une quelconque des revendications précédentes, dans lequel un agent de gravure utilisé lors de l'étape de gravure est l'hydroxyde de sodium, l'hydrogéno-carbonate de sodium ou le carbonate de sodium.

6. Procédé selon l'une quelconque des revendications précédentes, dans lequel le procédé après l'étape de gravure comprend une étape de teinture et/ou de teinture et impression.

7. Procédé selon l'une quelconque des revendications précédentes comprenant les étapes de préfixage, d'impression, de séchage, de fixage, de gravure, de savonnage, de teinture et de traitement final.
